

**1**

3,708,299

**PHOTOGRAPHIC DEVELOPING METHOD**

Isao Shimamura, Yoo Iijima, and Haruhiko Iwano, Kanagawa, Japan, assignors to Fuji Photo Film Co., Ltd., Kanagawa, Japan

No Drawing. Filed Oct. 8, 1970, Ser. No. 79,335

Claims priority, application Japan, Oct. 8, 1969,

44/80,538

Int. Cl. G03c 1/06, 5/26, 5/30

U.S. Cl. 96—66.3

8 Claims

**ABSTRACT OF THE DISCLOSURE**

A method and composition for processing a silver halide black and white photographic material wherein the silver halide grains are less than 0.3 micron which comprises developing the photographic material with a developing solution comprising hydroquinone (substituted or unsubstituted) as the main developing agent and imidazole in a minor amount.

**BACKGROUND OF THE INVENTION**

This invention relates to the processing of silver halide photographic materials and more particularly to developing solution for fine grained photographic materials.

**Description of prior art**

The desirable properties of processing procedures for silver halide, Black and White photographic materials reside in increased speed, high rate of development and fine grained silver image. The well known development accelerators are amine compounds, such as alkylamines (U.S. Pat. No. 2,196,037), aralkylamines (U.S. Pat. No. 2,496,903; 2,515,147; 2,541,889), phenoxyalkylamines (U.S. Patent No. 2,482,546), heterocyclic alkylamines (U.S. Pat. 2,605,183), morpholine and piperidine (U.S. Pat. No. 1,086,681). These amines, however, are poisonous, odoriferous and volatile, thus necessitating careful handling. Furthermore, their concentration in developing solution is often difficult to keep constant. The increase in rate of development is observed to some extent by an addition of these compounds to the developing solution, but this effect is often negated by the increase in fog formation. Furthermore, the deterioration in the granularity of the developed silver is often observed.

**SUMMARY OF THE INVENTION**

Therefore, the principal object of this invention is to provide an improved accelerator for the developing solution, which is easily handled, capable of increasing the rate of development and increasing the effective speed of the photographic material without undesirable increase in fog and the deterioration in the granularity of the developed silver.

Still another object of this invention is to provide a process for accelerating the developing of the fine grained photographic materials without deterioration in the granularity of the developed silver.

The developing solution of this invention is applied to the black-and-white photographic materials, especially to low sensitivity silver halide photographic materials which require fine granularity and is generally used for the office works, documentary works, industrial works, or reprographic works.

The present invention can be applied to telephotographic materials; lithographic materials (used for producing dots), phototypesetting materials, microfilms, microplates, materials for facsimile, materials for prints of scanned dots, materials for production of integral circuit master and photographic materials for astronomical study; these

**2**

photographic materials are composed of extremely fine grained silver halide and contain very small amounts of silver halide.

Therefore, these two features of the photographic materials provide different ways of development from that for the ordinary photographic materials.

For these materials, the granularity of the developed silver image should be adequately low throughout the development in the development of, e.g., fine grain silver halide emulsions as in the developing acceleration of this invention.

**Detailed description of the invention**

Accordingly, the present invention provides a method of treating a photographic material which comprise developing the materials with the developer containing imidazole and hydroquinone (substituted or unsubstituted) thus increasing the rate of development or shortening the developing time, inhibiting the fog formation, increasing the effective sensitivity and making fine the developed silver particles.

It has already been shown in U.S. Pat. No. 3,126,282 to add an imidazole to the first developer for the reversible color film whose emulsion contains non-diffusible color coupler to increase the speed of the film.

However, the increase in speed of the black-and-white photographic material to which this invention is applied by the imidazole is much greater than that of the reversible color film described in the U.S. Pat. 3,126,282. From 30 the examples of the specification, the reversible color film of this is considered to be composed of an emulsion of coarse silver iodobromide particles, while the emulsion of the Black and White photographic materials used in this invention contains finely divided silver halide particles.

That is to say, the process for developing the photographic material containing fine grain silver halides according to this invention has been made on a discovery that the increase in speed by an imidazole depends on the 40 size of the silver halide grain.

The fact that the developing of the photographic material with fine grain silver halides is accelerated by the imidazole when added to the developing solution in an amount contemplated herein has been unknown and have not been heretofore shown in the prior art. The expression "fine grained" denotes a particle size of from 0.1 to 0.3 micron.

**Preferred embodiments**

The developing solution exhibiting the aforesaid advantageous effects with the addition of the imidazole contains at least 1-20 parts/liter hydroquinone as the main developing agent and, in addition, a conventional developer such as 1-phenyl-3-pyrazolidone or N-methyl-p-aminophenol. If necessary, an oxidation inhibitor, such as Na sulfite or ascorbic acid, a suitable pH buffer, such as boric acid, sodium hydroxide, sodium carbonate or sodium phosphate, a developing inhibitor such as potassium iodide or potassium bromide, an organic fog inhibitor such as 6-nitro-benzimidazole or benzotriazole, and an aldehyde such as formaldehyde or glutaraldehyde can be added to the developing solution. The pH of this developing solution may be adjusted in a range between 8.5 and 12.0 and preferably 10 to 11. The amounts of the imidazole to be added to the developing solution vary with the type of the photographic material employed and the pH of the developing solution, but favorably in the range of between 0.5 part/liter and 100 parts/liter. The finely divided silver halide is present in a concentration of from 10-70 mg./100 cm.<sup>2</sup> and preferably 20-50 mg./cm.<sup>2</sup>.

A better understanding of the present invention will be had from the following examples which are merely illus-

trative and not limitative in nature. All parts are by weight unless otherwise stated.

## EXAMPLE 1

The 8 types of photographic films (I)-(VIII) were exposed to light by sensitometer and subjected to process of this invention; (I) commercial direct X-ray film, (II) high speed black and white negative film (ASA 100) for amateur use, (III) reversal color film (ASA 100) for amateur use, (IV) color negative film (ASA 100) for amateur use, (V) black and white fine grain posifilm for the cinematography, (VI) resographic film for photo-mechanical use, (VII) telephotographic film, (VIII) microfilm.

The process of this invention was not effective for the films (I)-(IV), but the test results were shown to be compared with those of the films (V)-(VII). The mean diameter of the silver halide grains in each of the photographic films were as follows:

| Photographic film: | Mean diameter of the silver particle, microns |
|--------------------|-----------------------------------------------|
| I                  | 1.4                                           |
| II                 | 0.8                                           |
| III                | 0.9                                           |
| IV                 | 1.0                                           |
| V                  | 0.15                                          |
| VI                 | 0.2                                           |
| VII                | 0.2                                           |
| VIII               | 0.2                                           |

Each of the photographic film (I)-(VII) was subjected to the developing treatment with the suitable developing solution below.

| Parts                                                 |
|-------------------------------------------------------|
| N-methyl-p-aminophenol ----- 5.0                      |
| Sodium sulfite ----- 70.0                             |
| Hydroquinone ----- 2.0                                |
| Sodium carbonate monohydrate ----- 41.0               |
| Potassium bromide ----- 4.0                           |
| Potassium thiocyanate ----- 1.6                       |
| Potassium iodide (0.1% aq. solution) (by vol.)-- 10.0 |

Water to make 1 liter.

(d) The developing solution for the photographic film (IV) (developer for the color negative film):

| Parts                                                                           |
|---------------------------------------------------------------------------------|
| Sodium hexamethaphosphate ----- 1.4                                             |
| Benzylalcohol ----- (by vol.)-- 5.0                                             |
| Sodium sulfite ----- 3.0                                                        |
| Sodium carbonate ----- 41.0                                                     |
| Sodium hydroxide ----- 1.0                                                      |
| 4-amino - 3 - methyl-N-ethyl-N-methane sulfonamidethylaniline sulfate ----- 5.0 |
| Potassium bromide ----- 0.5                                                     |

Water to make 1 liter.

(e) The developing solution for the photographic films (V)-(VIII):

"D-16" developing solution for the black and white posifilm (Eastman Kodak).

This "D-16" developer was also applied to the films (I) and (II), though they were processed by the developers (a) and (b), too. In the first series of the developing solutions (a)-(e) imidazole was not added and the second series 2.0 parts/liter added.

The test results were shown in the following table:

| Photographic films | Developing conditions (developer, temp., time) | Addition of imidazole, g./l. | Relative sensitivity (logarithmic sensitivity) | Notes                                               |
|--------------------|------------------------------------------------|------------------------------|------------------------------------------------|-----------------------------------------------------|
| I                  | "Rendol," 24° C., 5 min.                       | 0                            | 2.60                                           |                                                     |
| I                  | do                                             | 2.0                          | 2.65                                           | Increase in fog, deterioration of the silver image. |
| II                 | "D-76," 24° C., 6 min.                         | 0                            | 2.20                                           |                                                     |
| II                 | do                                             | 2.0                          | 2.30                                           | Deterioration of the silver image.                  |
| III                | (e), 24° C., 6 min.                            | 0                            | 2.35                                           |                                                     |
| III                | do                                             | 2.0                          | 2.50                                           | Do.                                                 |
| III                | (e) 1 24° C., 6 min.                           | 2.0                          | 2.45                                           |                                                     |
| IV                 | (d), 24° C., 10 min.                           | 0                            | 2.05                                           |                                                     |
| I                  | "D-16," 24° C., 5 min.                         | 0                            | 2.45                                           |                                                     |
| I                  | do                                             | 2.0                          | 2.10                                           |                                                     |
| II                 | do                                             | 2.0                          | 2.50                                           | Increase in fog, deterioration of the silver image. |
| II                 | do                                             | 0                            | 2.35                                           |                                                     |
| V                  | do                                             | 2.0                          | 2.45                                           | Deterioration of the silver image.                  |
| V                  | do                                             | 0                            | 0.25                                           |                                                     |
| VI                 | do                                             | 2.0                          | 1.00                                           |                                                     |
| VI                 | do                                             | 0                            | 1.05                                           |                                                     |
| VI                 | do                                             | 2.0                          | 1.45                                           |                                                     |
| VII                | do                                             | 0                            | 1.20                                           |                                                     |
| VII                | do                                             | 2.0                          | 1.60                                           |                                                     |
| VII                | do                                             | 0                            | 0.15                                           |                                                     |
| VII                | do                                             | 2.0                          | 1.05                                           |                                                     |

<sup>1</sup> (c) is a developing solution same as the (e) except for the lack of potassium thiocyanate.

(a) The developing solution for the photographic film (I):

Parts

|                                    |     |
|------------------------------------|-----|
| Mono-methyl-p-amino phenol -----   | 4.0 |
| Sodium sulfite (anhydride) -----   | 60  |
| Hydroquinone -----                 | 10  |
| Sodium carbonate (anhydride) ----- | 53  |
| Potassium bromide -----            | 2.5 |

Water to make one liter.

\*\*"Rendol" developing solution (produced by Fuji Photo Film Co., Ltd.)

(b) The developing solution for the photographic film (II):

"D-76" developing solution (produced by Eastman Kodak Co., Ltd.).

(c) The developing solution for the photographic film (III) (first developer for the reversal color film):

\*Mono-methyl-p-amino phenol—4.0 parts; sodium sulfite (anhydride)—60 parts; hydroquinone—10 parts; sodium carbonate (anhydride)—53 parts; potassium bromide—2.5 parts; water to make one liter.

It is apparent from this table that the addition of imidazole is very effective for the emulsion of fine grained silver halide.

## EXAMPLE 2

Commercial fine grain positive film for the cinematography composed of grained silver bromochloride-gelatin-emulsion was subjected to development with solution having following composition at 27° C.

## Developing solution A:

Parts

|                                      |                 |
|--------------------------------------|-----------------|
| Water -----                          | (by vol.)-- 800 |
| N-methyl-p-aminophenol sulfate ----- | 2.0             |
| Sodium sulfite -----                 | 100             |
| Hydroquinone -----                   | 5               |
| Borax -----                          | 2               |

Water to make 1 liter.

70 This developing solution required 4 min. to develop the positive film, but the addition of imidazole shortened the developing time substantially. On the other hand, 4 min. developing treatment with the imidazole added developing solution increased high sensitivity as shown in Table 1.

5  
TABLE 1

| Adding amounts (g./l.) | In 4 min. developing relative sensitivity Fog $\gamma$ |      |      | Developing time required to obtain relative sensitivity of 100 (min.) |
|------------------------|--------------------------------------------------------|------|------|-----------------------------------------------------------------------|
|                        | 100                                                    | 0.04 | 1.30 |                                                                       |
| Control-----           | 0                                                      | 100  | 0.04 | 1.30                                                                  |
| Imidazole-----         | 1                                                      | 180  | 0.04 | 1.33                                                                  |
| Do-----                | 4                                                      | 300  | 0.05 | 1.36                                                                  |

## EXAMPLE 3

A high resolution plate, comprising a support with ultra-fine grain silver iodobromide gelatin emulsion coated thereon was subjected to development at 20° C. with developing solution having following composition.

## Developing solution C:

|                                                             | Parts |
|-------------------------------------------------------------|-------|
| Water ----- (by vol.)                                       | 800   |
| 1-phenyl-3-pyrazolidone -----                               | 0.5   |
| Sodium sulfite -----                                        | 50    |
| Hydroquinone -----                                          | 12    |
| Sodium carbonate (NaCO <sub>3</sub> H <sub>2</sub> O) ----- | 60    |
| Potassium bromide -----                                     | 2.0   |
| Benzotriazole -----                                         | 0.2   |
| Water to make 1 liter.                                      |       |

This developing solution required 6 min. to develop the dry plate, but the imidazole added developing solution shortened the developing time as shown in Table 2. On the other hand, 6 min. of development with the imidazole containing developing solution exhibited high sensitivity on the dry plate.

TABLE 2

| Adding amounts (parts/l.) | In 4 min. developing relative sensitivity Fog $\gamma$ |      |      | Developing time required to obtain the relative sensitivity 100 |
|---------------------------|--------------------------------------------------------|------|------|-----------------------------------------------------------------|
|                           | 100                                                    | 0.04 | 3.24 |                                                                 |
| Control-----              | 0                                                      | 100  | 0.04 | 3.24                                                            |
| Imidazole-----            | 1                                                      | 150  | 0.04 | 3.40                                                            |
| Do-----                   | 2                                                      | 280  | 0.05 | 3.75                                                            |

## EXAMPLE 4

Commercial microfilm comprising a support with a fine grain silver chlorobromide, gelatin emulsion coated thereon, was subjected to development at 20° C. with a developing solution having following composition.

## Developing solution E:

|                                                             | Parts |
|-------------------------------------------------------------|-------|
| Water ----- (by vol.)                                       | 800   |
| N-methyl-p-aminophenol sulfate -----                        | 1.0   |
| Sodium sulfite -----                                        | 75    |
| Hydroquinone -----                                          | 9.0   |
| Sodium carbonate (NaCO <sub>3</sub> H <sub>2</sub> O) ----- | 29    |
| Potassium bromide -----                                     | 6.0   |
| Water to make 1 liter.                                      |       |

The developing solution of E required 4 minutes to develop the microfilm, but the addition of the imidazole to the developing solution shortened the developing time as shown in Table 3. On the other hand, a development time of 4 minutes with the imidazole added to the developing solution produced a high sensitivity on the microfilm. Furthermore, the developed silver grains in the picture were favorably fine and uniform according to the process of this invention using the imidazole containing developing solution.

6  
TABLE 3

| 5              | Adding amounts (parts) | In 4 min. developing relative sensitivity Fog $\gamma$ |      |      | Developing time (min.) required to obtain the relative sensitivity 100 |
|----------------|------------------------|--------------------------------------------------------|------|------|------------------------------------------------------------------------|
|                |                        | 100                                                    | 0.19 | 4.00 |                                                                        |
| Control-----   | 0                      | 100                                                    | 0.19 | 4.00 | 4                                                                      |
| Imidazole----- | 1                      | 140                                                    | 0.20 | 4.06 | 3                                                                      |
| Do-----        | 4                      | 250                                                    | 0.21 | 4.08 | 2                                                                      |

10 Said results have been attained wherein the silver halide contains fine grained silver chlorobromide and less than 1% of silver iodide, the particle size being smaller than 0.2 micron.

15 As this invention has been particularly illustrated with reference to the examples, it will be clearly understood to one skilled in the art that the scope of this invention is not to be restricted to the examples and claims but that various alterations and modifications may be made without departing from the spirit of this invention.

20 Similar results have also been achieved using substituted hydroquinones and specifically, chloro, bromo, methyl, dimethyl, phenyl and methyl phenyl.

What is claimed is:

25 1. A method for processing an exposed silver halide black-and-white photographic material, wherein the silver halide grains are less than 0.3 micron which comprises developing the photographic material with a developing solution comprising at least 1.0 part of hydroquinone as the main developing agent and at least 0.5 part of imidazole per one liter of the developing solution.

30 2. The method of claim 1, wherein the concentration of hydroquinone and imidazole respectively is 1.0-20 grams/l. and 0.5-10.0 grams/l. by weight.

35 3. The method of claim 2, wherein the concentration of imidazole is from 1.0-6.0 grams/l.

40 4. The method of claim 1, wherein the size of the silver halide particles is less than 0.2 micron.

45 5. The method of claim 1, wherein the pH range is between 8.5 and 12.

60 6. The method of claim 5, wherein the pH ranges from 10-11.

7. The method as claimed in claim 1, wherein said silver halide contains fine grain silver chlorobromide and less than 1% of silver iodide, particle size of said silver halide being smaller than 0.2 micron.

45 8. The method of claim 5, wherein the silver halide is present in a range of from 10-70 mg./100 cm.<sup>2</sup>.

## 50 50 References Cited

## UNITED STATES PATENTS

|           |         |                     |         |
|-----------|---------|---------------------|---------|
| 2,324,123 | 7/1943  | Weissberger -----   | 96—66.5 |
| 2,605,183 | 7/1952  | Runyan -----        | 96—66.3 |
| 3,046,130 | 7/1962  | Dersch et al. ----- | 96—67   |
| 3,086,863 | 4/1963  | Hunt et al. -----   | 96—108  |
| 3,126,282 | 3/1964  | Hunt -----          | 96—59   |
| 3,271,154 | 9/1966  | Dersch et al. ----- | 96—66   |
| 3,335,009 | 8/1967  | Rasch et al. -----  | 96—61   |
| 3,353,956 | 11/1967 | Rogers et al. ----- | 96—29   |
| 3,397,987 | 8/1968  | Luckey et al. ----- | 96—109  |
| 3,576,633 | 4/1971  | Henn et al. -----   | 96—66.5 |

65 J. TRAVIS BROWN, Primary Examiner

M. F. KELLEY, Assistant Examiner

U.S. Cl. X.R.

96—50 R, 66 R, 66.5, 95